

## UNITED STATES PATENT OFFICE

FREDERICK R. BYROD, OF SUNBURY, PENNSYLVANIA, ASSIGNOR TO SUSQUEHANNA  
SILK MILLS, A CORPORATION OF NEW YORK

## COLOR DISCHARGE PRINTING

No Drawing.

Application filed December 10, 1931. Serial No. 580,224.

The present invention relates to a process of color discharge printing and to the colored discharge printing pastes employed therein. The process is applicable to any textile fabric, whether of animal or vegetable origin. It is particularly suitable for silk and rayon fabrics. It has hitherto been customary to prepare colored discharges by printing a fabric which has been dyed with a reducible ground color by means of a paste comprised of a reducing agent, such as hydrosulfite, formaldehyde-sulfoxylate, or other combinations of hydrosulfite and formaldehyde, etc., a coloring matter which is unaffected by the reducing agent and one of the usual thickeners, such as gums, dextrines and the like. The reducing agents are found on the market under various trade names, such as Rongalite, Discolite, Sulfoxite and Hydrosulphite, A. W. C. This process was not fully satisfactory because when printing medium and pastel shade intensities is attempted, the resultant shade on silk, rayon and the like has a tendency to show a washed out character, sometimes changing in cast or color, as, for instance, from a luminous medium blue to a washed out greenish blue. There is also the difficulty of unevenness in so far as given surfaces have a tendency to show white rings around the area where the colored mixture of reducing agent thickener and unreducible dye has been applied. Sometimes a mottled or speckled appearance develops. Again there exists the constant risk of irregularity of developing finely fixed tones in the aging process, which, in many cases, causes the same coloring matter made with identical formulas to appear in successive printings either dark, medium or sometimes so light that for all practical purposes it has disappeared. The latter effect has never been definitely accounted for, but it is commonly known that it is as good as impossible to keep a definite cast of color on silk which passes through the aging process.

I have found that these disadvantages can almost completely be avoided in a very simple manner. According to my new process a substantial amount of finely divided titanium dioxide is added to the colored discharge paste. The titanium dioxide, thus added, may serve to replace part of the thickening agent formerly used in the preparation of the colored discharge paste. The essential constituents of my improved colored discharge paste are a reducing agent, such as hydrosulfite, formaldehyde-sulfoxylate, or other combinations of hydrosulfite and formaldehyde and the like, a coloring matter which is unaffected, i. e., not reduced, by the reducing agent and titanium dioxide. Further additions, such as are customary in the preparation of printing paste, may also be present, such as thickeners, glycerine, etc. One may substitute zinc oxide for part of the titanium dioxide, and this will in most cases be advisable, owing to the higher cost of the titanium dioxide. However, the quality of the colored prints obtained is improved by the use of a greater proportion of the titanium dioxide and, therefore, a substantial amount thereof is always used in the preparation of my improved colored discharge pastes. The titanium dioxide present in the colored discharge pastes has a delustering effect on rayon, which makes the color stand out. Thus, the quality of the colored prints obtained is improved by the delustering effect of the titanium dioxide present and the possibility of mechanical defects during the printing process is strongly reduced by the presence of a substantial proportion of titanium dioxide in the colored discharge paste.

The amount of the titanium dioxide, or mixture of titanium dioxide and zinc oxide, present in the colored discharge paste may vary within wide limits. Preferably it will constitute from 3 percent to 24 percent by weight of the colored discharge paste.

The particular coloring matters suitable for use in the process can readily be selected by those skilled in the art. As has been pointed out above, the ground color should consist of a dischargeable, i. e., reducible, dyestuff, whereas the coloring matter contained in the colored discharge paste should consist of the dyestuff which is unaffected, i. e. not

100

reduced, by the reducing agent present in the paste.

As typical examples of such dyestuffs the following may be mentioned:

5

*Dischargeable ground colors*

DIRECT COLORS

| 10 | Name of color         | Rowe's Color Index No. | Schultz No. |
|----|-----------------------|------------------------|-------------|
| 15 | Amanil blue 2B        | 406                    | 337         |
|    | Chloramine red 3B     | 382                    | 319         |
|    | Direct black          | 531                    | 462         |
|    | Direct blue 3B        | 477                    | 391         |
|    | Direct green B        | 593                    | 474         |
|    | Direct sky blue FF    | 518                    | 424         |
|    | Eris fast brown GR    | 598                    | 477         |
|    | Eris fast scarlet YA  | 326                    | 279         |
|    | Fast acid green B     | 667                    | 503         |
|    | Triazol yellow G      | 365                    | 304         |
| 20 | DEVELOPED COLORS      |                        |             |
| 25 | Diazamine blue BR     | 316                    | 273         |
|    | Diazo black BH        | 401                    | 333         |
|    | Diazo fast green BL   | 532                    |             |
|    | Diazol fast violet NN | 394                    | 327         |
|    | Diazo indigo blue B   | 316                    | 273         |
|    | Plutoform black L     | 545                    |             |
|    | Rosanthrene O         | 324a                   |             |

*Non-dischargeable print colors*

BASIC COLORS

|    |                         |     |     |
|----|-------------------------|-----|-----|
| 30 | Euchrysine RDX          | 797 | 608 |
|    | Methylene blue B        | 922 | 659 |
|    | Nigrosine water soluble | 865 | 700 |
|    | Nile blue B             | 914 | 654 |
|    | Phosphine O Ex          | 793 | 606 |
|    | Rhodamine B Ex          | 749 | 573 |
| 35 | Rhodamine 6G Ex         | 752 | 571 |
|    | Rhoduline blue GO       | 926 | 661 |
|    | Safranine A             | 841 | 679 |
|    | Thioflavine T           | 815 | 618 |

ACID COLORS

|    |                |     |     |
|----|----------------|-----|-----|
| 40 | Azo carmine GX | 828 | 672 |
|----|----------------|-----|-----|

VAT COLORS

|    |                                 |      |     |
|----|---------------------------------|------|-----|
| 45 | Algol scarlet G                 | 1129 | 815 |
|    | Anthrene jade green             | 1101 |     |
|    | Ciba orange G                   | 1230 | 911 |
|    | Ciba scarlet G Dbl. paste pat   | 1228 | 907 |
|    | Indanthrene black B             | 1102 | 765 |
|    | Indanthrene blue GCD Dbl. paste | 1113 | 842 |
|    | Indanthrene yellow G Dbl. paste | 1118 | 849 |

50 The following are examples of discharge pastes to which the unreduceable printing color may be added (parts by weight):

A

| 55 |                     | Grams |
|----|---------------------|-------|
|    | Titanium dioxide    | 49    |
|    | Zinc oxide          | 84    |
|    | Glycerine           | 71    |
|    | Olive oil           | 20    |
| 60 | Water               | 138   |
|    | Textile gum         | 265   |
|    | Hydrosulphite (1:1) | 280   |
|    | Egg albumen (1:1)   | 93    |
| 65 | Total               | 1,000 |

| B                          |        |
|----------------------------|--------|
| Titanium dioxide           | 140    |
| Zinc oxide                 | 32     |
| Glycerine                  | 72 70  |
| Olive oil                  | 20     |
| Water                      | 130    |
| Textile gum                | 165    |
| Hydrosulphite 50% solution | 248    |
| Egg albumen 50% solution   | 193 75 |
| Total                      | 1,000  |

C

|                            |        |
|----------------------------|--------|
| Titanium dioxide           | 178 80 |
| Zinc oxide                 | 0      |
| Glycerine                  | 81     |
| Olive oil                  | 25     |
| Water                      | 162    |
| Textile gum                | 118 85 |
| Hydrosulphite 50% solution | 210    |
| Egg albumen 50% solution   | 226    |
| Total                      | 1,000  |

The discharge printing process is carried out in the usual manner. The textile material, for example, a silk or rayon fabric, is first dyed with the reducible ground color. It is then printed in the usual manner with the colored discharge paste. Thereupon the material is developed, for example, by steaming in a Mather-Platt apparatus, and finally washed and soaped.

Obviously my invention is not limited to the particular examples given above. As has already been pointed out, the crux of my invention resides in the use of titanium dioxide as one of the constituents of the colored discharge paste used.

I claim:

1. A process of obtaining colored discharges on textile materials which have been dyed with a dischargeable ground color which comprises printing said materials with a colored discharge paste containing a reducing agent, an unreduceable coloring matter and titanium dioxide.

2. A process of obtaining colored discharges on textile materials which have been dyed with a dischargeable ground color which comprises printing said materials with a colored discharge paste containing a reducing agent of the group consisting of hydrosulfite, formaldehyde-sulfoxylate and other combinations of hydrosulfite and formaldehyde, an unreduceable coloring matter and from 3 percent to 24 percent by weight of titanium dioxide.

3. A process of obtaining colored discharges on textile materials which have been dyed with a dischargeable ground color which comprises printing said materials with a colored discharge paste containing a reducing agent, an unreduceable coloring matter, titanium dioxide and zinc oxide.

4. A process of obtaining colored discharges on textile materials which have been dyed with a dischargeable ground color which comprises printing said materials with a colored discharge paste containing a reducing agent of the group consisting of hydro-sulfite, formaldehyde-sulfoxylate and other combinations of hydrosulfite and formaldehyde, an unreduceable coloring matter and from 3 percent to 24 percent by weight of titanium dioxide and zinc oxide.

5. A process of obtaining colored discharges on silk fabrics which have been dyed with a dischargeable ground color which comprises printing said fabrics with a colored discharge paste containing hydrosulfite, a dyestuff which is not reduced by the hydrosulfite, and from 3 percent to 24 percent by weight of titanium dioxide and zinc oxide, developing said fabrics by steaming and then 10 washing and soaping the fabrics.

6. A colored discharge paste which comprises a reducing agent and unreduceable coloring matter and titanium dioxide.

7. A colored discharge paste which comprises a reducing agent of the group consisting of hydrosulfite, formaldehyde-sulfoxylate and other combinations of hydrosulfite and formaldehyde, an unreduceable coloring matter and from 3 percent to 24 percent by 20 weight of titanium dioxide.

8. A colored discharge paste which comprises a reducing agent, an unreduceable coloring matter, titanium dioxide and zinc oxide.

35 9. A colored discharge paste which comprises a reducing agent of the group consisting of hydrosulfite, formaldehyde-sulfoxylate and other combinations of hydrosulfite and formaldehyde, an unreduceable coloring matter and from 3 percent to 24 percent by weight of titanium dioxide and zinc oxide.

40 10. A colored discharge paste which comprises hydrosulfite, a dyestuff which is not reduced by the hydrosulfite and from 3 percent to 24 percent by weight of titanium dioxide and zinc oxide.

45 In testimony whereof I have hereunto set my hand.

FREDERICK R. BYROD.